

## UNITED STATES PATENT OFFICE

2,576,922

## ELECTRODEPOSITION WITH NICKEL

Etienne L. A. Camin, New York, N. Y., and Sven E. Hybinette and Herbert B. Taylor, Wilmington, Del., assignors, by mesne assignments, to Kenmore Metals Corporation, a corporation of Delaware

No Drawing. Application June 26, 1946,  
Serial No. 679,558

12 Claims. (Cl. 204—49)

**1**  
This invention relates to the art of electrodeposition and is directed particularly to a process and to a bath for the electrodeposition with nickel.

This application is a continuation-in-part of application Serial No. 446,819, filed June 12, 1942, now abandoned.

An object of this invention is to produce a ductile nickel plating on metal which can be drawn. The ductility of the product obtainable by the process of this invention goes considerably beyond the previous standards of ductility in this art. For example, a plated article is considered ductile if it can be hammered or bent without cracking. According to the present invention, plated articles may be made in which the product is so ductile that it may be drawn several thousands of times its previous length and the drawn product can still be bent, twisted or braided without causing the plating to crack.

Another object of this invention is to produce a nickel plating bath from nickel or nickel salts, hydrofluoric acid and a buffering agent which has substantially the same throwing power as a sulphate-chloride type of nickel plating bath.

Another object of this invention is to expedite the rate of electrodeposition of nickel and at the same time attain generally improved operating characteristics.

Another object of this invention is to produce a bath which stays indefinitely in condition for plating with very little control other than replenishment with water and with a small amount of fresh bath prepared to compensate for losses by "drag out."

Another object of this invention is to produce a deposit of nickel on metal with uniform properties throughout the entire deposit.

Another object of the present invention is to produce heavy deposits of nickel on metal in smooth condition by employing a process and a bath in which the nickel does not "tree" as heavily as in the prior art.

These and other objects ancillary thereto are obtained by making up a bath of nickel, hydrofluoric acid and a buffer in which the various proportions of the ingredients are critical and in employing this bath to attain specified conditions set forth below to produce the smooth and/or ductile nickel deposit or plating.

In general the following proportions and conditions are important in the practice of this invention:

1. The amount of nickel in the bath should be at least 30 grams per liter. The upper limit of the nickel content is determined partly by the temperature employed; the higher the temperature the less stable or soluble is the nickel salt. The amount of nickel is also limited by

the pH of the bath, more nickel being soluble at the lower pH values. Thus, the upper limit of nickel content of the bath is determined mainly by the solubility of the nickel or nickel salt. Generally a high nickel content favors the production of a ductile plate at high current densities. With a low nickel content, such as for example about 30 grams per liter, low current densities must be employed which might be uneconomical for commercial production. However, a satisfactory plate may be obtained at a slightly lower nickel content.

2. The buffer employed in the bath is preferably boric acid although it is quite possible that other buffers, such as the more expensive citric acid or tartaric acid, could be employed. The boric acid besides acting as a buffer also reacts with the nickel ion in the bath to produce a complex nickel salt possibly a fluoroborate. Thus, it is preferable to add some excess of the boric acid over that required to react with the nickel in the bath. The range of the boric acid necessary is from about 20 to over 60 (depending on the solubility) grams per liter. The presence of the buffer increases the stability of the bath.

3. In making up the bath hydrogen fluoride is preferably employed although the addition of a fluoride ion from another source is not excluded. Apparently the hydrofluoric acid reacts with the nickel and boric acid in the bath to produce the aforementioned complex nickel salt. The hydrofluoric acid is employed in excess so as to produce the desired pH which is on the acid side.

We have also found that the boric acid content should be relatively high not only by reason of its ordinary buffer action but because it improves anode corrosion, lowers the tendency of heavy deposits to form "trees," and produces a more ductile deposit.

4. The hydrogen ion concentration or pH of the bath is important and generally must be maintained between a pH 1 and a pH 6. At the pH values of close to 6 there is less tolerance permissible on the other conditions maintained in the bath. Also at the higher pH, such as about 6 or above, hydroxyl inclusion in the plating may cause brittleness. The solubility of the nickel or nickel salt in the bath increases as the pH value is lowered. However, at around a pH 1, hydrogen inclusion in the plating may cause brittleness as hydrogen evolution is increased at lower pH values. At the lower pH values one obtains better anode corrosion and a smaller amount of buffer is necessary. At the higher pH values the ductility of the product is somewhat better.

5. The temperature of the bath is not extremely critical but it is noted that at the higher

temperatures the nickel salt tends to precipitate and at the lower temperatures the buffer or boric acid will tend to precipitate. Also the resistance of the bath decreases with increasing temperatures making a higher current density possible at the higher temperature. Although the nickel tends to precipitate at higher temperatures, with baths of low nickel content temperatures of as high as 75° C. may be used. It is preferred, however, to operate at temperatures between 40 and 70° C.

6. The range of current density which can be employed is wide. It is well known that the more intensive the agitation of the solution and/or the cathode, the higher is the current density which can be employed. Our invention enables us to employ current densities two to three times higher than generally is possible under the same conditions of agitation. (In the art, current density is always referred to the surface area of the cathode unless the anode is specified.) For the best ductility the current densities of from 3-50 amps. per square decimeter are advantageous. High current densities are known in one other type bath, i. e. the high chloride type bath. These baths have the disadvantages of having a very low pH and of being very corrosive and can only be used with special equipment and with special protection for the operation. For these reasons these baths have not gained wide popularity. The baths of the present invention do not suffer from these defects.

It is also sometimes advisable to add a wetting agent to the bath which minimizes the effect of the evolution of hydrogen on the plate and, therefore, aids in the production of a more ductile and pore-free plate. Mechanical vibrations may also be employed to minimize the effect of the evolution of hydrogen. An example of a wetting agent which may be used is "Duponol ME" which is a fatty alcohol sulphate type of wetting agent. Other wetting agents of this type or of any type which will stand up in an acid solution with a high salt content may be employed. Examples of such wetting agents are: quaternary ammonium compounds such as lauryl pyradonium chloride, long chain polyethylene oxide compounds such as "Carbowax," etc.

The following examples of plating baths and operating conditions in addition to those given above (the acidic pH values resulting from the excess of hydrofluoric acid) will serve to further illustrate the invention:

| Example | Ni, in g./l. | Boric acid in g./l. | Current density in amp./dm. <sup>2</sup> | Temperature, in degrees C. | pH         |
|---------|--------------|---------------------|------------------------------------------|----------------------------|------------|
| 1       | 60           | 30                  | 25                                       | 50                         | 1          |
| 2       | 42           | 30                  | 15                                       | 45                         | 6.0        |
| 3       | 50           | 45                  | 1 to 50                                  | 60                         | 4 to 5     |
| 4       | 60           | 45                  | 1 to 250                                 | 60                         | 2.5 to 4   |
| 5       | 48           | 45                  | 120                                      | 60                         | 4.2        |
| 6       | 50           | 50                  | 250                                      | 60                         | 3.2        |
| 7       | 50           | 45                  | 15                                       | 60                         | 4          |
| 8       | 45           | 50                  | 20                                       | 50                         | 3.5        |
| 9       | 30           | 40                  | 1 to 12                                  | 60                         | 4.7 to 5.2 |
| 10      | 36           | 40                  | 1 to 15                                  | 60                         | 4.7 to 5.2 |
| 11      | 75           | 35                  | 1 to 250                                 | 50                         | 4.2 to 4.7 |
| 12      | 60           | 40                  | 15 to 25                                 | 70                         | 5.2        |

The examples with a pH of 1 produced somewhat brittle plates due to excessive evolution of hydrogen at the cathode. Using a pH of 6, the main difficulty is the keeping of the nickel in solution. The examples with a pH of 6 and above produced somewhat brittle plate.

It has been determined that nickel deposited in accordance with the present invention is re-

markably adherent to various metals and alloys even when deposited directly on such metals and alloys, that is to say, even in the absence of any preparatory plating. Among the various alloys on which we have plated nickel in accordance with this invention is, for example, steel. The plating of nickel directly on steel has always presented a difficult problem, inasmuch as good adherence and freedom from pits have always been very difficult to secure without special precautions, particularly when deposits greater than .0005" thick are required. It is common practice to first deposit copper on steel and then to deposit the nickel on the copper plating. However, by the use of the bath embodying the present invention no difficulty is encountered in producing on steel a plating which possesses remarkable adherence and is substantially free from pits even when the thickness of the plating greatly exceeds .0005". Thus, according to the process of this invention, one plating step is eliminated and the results achieved are at least as good as those obtainable by the double plating processes of the prior art.

In the foregoing examples, ductility was also determined by making plates .002" thick on copper wire and bending the plated wire over a rod four times the diameter of the wire. The plate at the bend was dipped first in hydrochloric acid and then in sodium polysulphide, and then examined under a microscope. If no cracks were revealed there was considered to be a good ductile plate.

A  $\frac{1}{16}$ " diameter steel wire plated according to Example 12 with 5% by weight of nickel and at a current density of 25-30 amperes per square decimeter was drawn from a length of 3 feet to 16,000 feet and in every stage of the drawing could be bent, flexed, twisted or otherwise worked. The drawn wire still contained 5% by weight of nickel as determined by chemical analysis. The resultant drawn wire was also more resistant to corrosion due to the fact that in the drawing process the nickel plating became denser and at the same time retained its continuity.

A 1" (outside diameter) brass tube plated with 10% by weight of nickel according to the process of Example 3 (above) with a current density of about 30 amps. per square decimeter was drawn to  $\frac{1}{16}$ " and the plating showed no signs of cracking.

We believe that the degree of ductility achieved by the present invention is due to the crystal structure of the nickel deposit. X-ray tests seem to show that the nickel crystals deposited from our bath are not deposited one alongside the other in the form known as "trees" but that a sufficient number of the crystals are aligned parallel to the surface of the base material to form brick-like layers and that these layers "flow" with the base metal when drawn, whereas a normal crystal growth perpendicular to the surface of the base metal separates when the plating is drawn.

The tendency of nickel to become passive when employed in an electroplating anode is well known and is highly objectionable in that it commonly causes the nickel anode to corrode unevenly and in that it prompts the undue release from the anode of metallic particles. These particles, aside from representing a loss of nickel, often fall on the work being plated and cause blemishes in the plate. By the use of specially compounded and treated anodes, uneven corrosion of the anode and the undue release of metallic particles there-

from may be minimized, but such compounding and treatment of the anodes is obviated when a bath embodying the present invention is employed, inasmuch as the anode nickel does not become passive in such bath. Actually, the bath is such that we can satisfactorily use pure, hard-rolled, fine-grained nickel or ordinary "cathode sheets" as an anode, devoid of any special compounding or treatment as heretofore required.

Inasmuch as the bath embodying the present invention contains an excess of hydrofluoric acid, it becomes necessary to employ tanks or vessels which are resistant to this acid. Vitreous tanks and wood vessels should be avoided, but hard rubber or rubber coated steel may be used to advantage. Vitreous tanks, however, are usable with a high pH.

Nickel plating baths in common usage cannot hold much iron in solution with the result that if any appreciable amount of iron is introduced it will be precipitated. Most nickel anodes contain some iron which enters the solution continuously, only to be precipitated. It has heretofore often been found necessary to constantly filter the solution or provide a very deep electroplating tank so that the iron precipitate may settle to such a depth in the bath as to obviate the danger of its being stirred up during the carrying out of the plating process. By use of my improved electroplating bath, all iron entering into the solution from the anode (assuming the anode is primarily nickel and contains some iron) will remain in solution, thus obviating the formation of an iron precipitate. During the course of the electroplating operation, the iron in solution will be plated out with the nickel and deposited on the cathode. Thus, it will be understood that iron may, by design, be added to the solution for the purpose of producing a plate consisting of a nickel iron alloy. In such a case, certain of the anodes would be constituted of iron. Likewise, the bath is such in its operation that cobalt may be intentionally introduced in the solution when an electrodeposition of cobalt is desired along with the nickel.

Several courses are available for the preparation of the bath. It can be prepared, for example, by dissolving solid commercial nickel carbonate in hydrofluoric acid or by electrolyzing hydrofluoric acid with nickel anodes. While in the claims reference is made to the nickel being present in the form of nickel fluoride, it will be understood that actually nickel will be present largely in the form of complex salts including nickel fluoborates. Accordingly, it is contemplated that the term nickel fluoride embraces complex nickel salts. The plating bath should be as pure as possible for high current densities. Thus, traces of lead if over .04 per cent which might enter the hydrofluoric acid from a lead container may lead to brittleness, flaking and bad appearance in general.

By the addition of known brightening agents such as, for example, a mixture of paratoluene sulfonamide, saccharine and fuchsin the baths of the present invention may be employed for producing bright plating and it is then possible to work with high current densities (up to 2 or more) compared to the commercial brightening baths. This possibility of working with high current densities is the important advantage in baths of the present invention where brightening agents are added since it is well known in the art that the addition of brightening agents to the electroplating baths reduces the ductility of the plating.

The particular bath employed when plating according to the present invention depends upon such factors as the ductility required, the rate of deposition required, and the character of the plating operations to be undertaken. The exact composition of the bath and the operating characteristics thereof for any particular set of requirements will be apparent to those skilled in the art.

We claim:

1. A method for producing a relatively ductile nickel plating on a metal base which comprises passing a current of less than 250 amperes per square decimeter from a nickel anode to the metal base to be plated through a bath formed essentially from a nickel compound, hydrofluoric acid, boric acid and water, said hydrofluoric acid reacting with said nickel compound to form a complex nickel fluoride, said hydrofluoric acid being present in a quantity in excess of that required to convert said nickel compound to said complex nickel fluoride, said bath containing at least 30 grams of nickel metal per liter, said excess hydrofluoric acid giving said bath a pH of more than 1 and less than 6, the anions of said bath comprising essentially fluorides and borates.

2. A method for producing a highly ductile nickel plating on a metal base which comprises passing a current of less than 250 amperes per square decimeter from a nickel anode to the metal base to be plated through a bath formed essentially from nickel carbonate, hydrofluoric acid, boric acid and water, said hydrofluoric acid reacting with said nickel carbonate to form a complex nickel fluoride, said hydrofluoric acid being present in a quantity in excess of that required to convert said nickel carbonate to said complex nickel fluoride, said bath containing at least 30 grams of nickel metal per liter, said excess hydrofluoric acid giving said bath a pH of more than 1 and less than 6, the anions of said bath comprising essentially fluorides and borates.

3. A method for producing a highly ductile nickel plating on a metal base which comprises passing a current of less than 250 amperes per square decimeter from a nickel anode to the metal base to be plated through a bath formed essentially from nickel, hydrofluoric acid, boric acid and water, said hydrofluoric acid reacting with said nickel to form a complex nickel fluoride, said hydrofluoric acid being present in a quantity in excess of that required to convert said nickel to said complex nickel fluoride, said bath containing at least 30 grams of nickel metal per liter, said excess hydrofluoric acid giving said bath a pH of more than 1 and less than 6, the anions of said bath comprising essentially fluorides and borates.

4. A method for producing a highly ductile nickel plating on a metal base which comprises passing a current of less than 250 amperes per square decimeter from a nickel anode to the metal base to be plated through a bath formed essentially from a nickel compound, hydrofluoric acid, boric acid and water, said hydrofluoric acid reacting with said nickel compound to form a complex nickel fluoride, said hydrofluoric acid being present in a quantity in excess of that required to convert said nickel compound to said complex nickel fluoride, said bath containing at least 30 grams of nickel metal per liter, and 20-60 grams of boric acid per liter, said excess of hydrofluoric acid giving said bath a pH of more than 1 and less than 6, the anions of said bath comprising essentially fluorides and borates.

5. A method for producing a highly ductile

nickel plating on a metal base which comprises passing a current of less than 250 amperes per square decimeter from a nickel anode to the metal base to be plated through a bath formed essentially from a nickel compound, hydrofluoric acid, boric acid and water, said hydrofluoric acid reacting with said nickel compound to form a complex nickel fluoride, said hydrofluoric acid being present in a quantity in excess of that required to convert said nickel compound to said complex nickel fluoride, said bath containing from 42 to 60 grams of nickel metal per liter, said excess hydrofluoric acid giving said bath a pH of more than 1 and less than 6, the anions of said bath comprising essentially fluorides and borates.

6. A method for producing a highly ductile nickel plating on a metal base which comprises passing a current of from 15 to less than 250 amperes per square decimeter from a nickel anode to the metal base to be plated through a bath formed essentially from a nickel compound, hydrofluoric acid, boric acid and water, said hydrofluoric acid reacting with said nickel compound to form a complex nickel fluoride, said hydrofluoric acid being present in a quantity in excess of that required to convert said nickel compound to said complex nickel fluoride, said bath containing at least 30 grams of nickel metal per liter, said excess hydrofluoric acid giving said bath a pH of more than 1 and less than 6, the anions of said bath comprising essentially fluorides and borates.

7. A method for producing a highly ductile nickel plating on a metal base which comprises passing a current of from 15 to less than 250 amperes per square decimeter from a nickel anode to the metal base to be plated through a bath formed essentially from a nickel compound, hydrofluoric acid, boric acid and water, said hydrofluoric acid reacting with said nickel compound to form a complex nickel fluoride, said hydrofluoric acid being present in a quantity in excess of that required to convert said nickel compound to said complex nickel fluoride, said bath containing from 42 to 60 grams of nickel metal per liter, said excess hydrofluoric acid giving said bath a pH of more than 1 and less than 6, the anions of said bath comprising essentially fluorides and borates.

8. A bath for the electrodeposition of a relatively ductile nickel coating on a metal base which is formed essentially from a nickel compound, hydrofluoric acid, boric acid and water, said hydrofluoric acid reacting with said nickel compound to form a complex nickel fluoride, said hydrofluoric acid being present in a quantity in excess of that required to convert said nickel compound to said complex nickel fluoride, said bath containing at least 30 grams of nickel metal per liter, said excess of hydrofluoric acid giving said bath a pH of more than 1 and less than 6, the anions of said bath comprising essentially fluorides and borates, said bath producing said relatively ductile nickel coating when operated at current densities of less than 250 amperes per square decimeter.

9. A bath for the electrodeposition of a highly ductile nickel coating on a metal base which is formed essentially from nickel carbonate, hydrofluoric acid, boric acid and water, said hydrofluoric acid reacting with said nickel carbonate to form a complex nickel fluoride, said hydrofluoric acid being present in a quantity in excess of that required to convert said nickel carbonate to said complex nickel fluoride, said bath containing at least 30 grams of nickel metal

per liter, said excess hydrofluoric acid giving said bath a pH of more than 1 and less than 6, the anions of said bath comprising essentially fluorides and borates, said bath producing said highly ductile nickel coating when operated at current densities of less than 250 amperes per square decimeter.

10. A bath for the electrodeposition of a highly ductile nickel coating on a metal base which is formed essentially from nickel, hydrofluoric acid, boric acid and water, said hydrofluoric acid reacting with said nickel to form a complex nickel fluoride, said hydrofluoric acid being present in a quantity in excess of that required to convert said nickel to said complex nickel fluoride, said bath containing at least 30 grams of nickel metal per liter, said excess hydrofluoric acid giving said bath a pH of more than 1 and less than 6, the anions of said bath comprising essentially fluorides and borates, said bath producing said highly ductile nickel coating when operated at current densities of less than 250 amperes per square decimeter.

11. A bath for the electrodeposition of a highly ductile nickel coating on a metal base which is formed essentially from a nickel compound, hydrofluoric acid, boric acid and water, said hydrofluoric acid reacting with said nickel compound to form a complex nickel fluoride, said hydrofluoric acid being present in a quantity in excess of that required to convert said nickel compound to said complex nickel fluoride, said bath containing at least 30 grams of nickel metal per liter, and 20-60 grams of boric acid per liter, said excess of hydrofluoric acid giving said bath a pH of more than 1 and less than 6, the anions of said bath comprising essentially fluorides and borates, said bath producing said highly ductile nickel coating when operated at current densities of less than 250 amperes per square decimeter.

12. A bath for the electrodeposition of a highly ductile nickel coating on a metal base which is formed essentially from a nickel compound, hydrofluoric acid, boric acid and water, said hydrofluoric acid reacting with said nickel compound to form a complex nickel fluoride, said hydrofluoric acid being present in a quantity in excess of that required to convert said nickel compound to said complex nickel fluoride, said bath containing from 42 to 60 grams of nickel metal per liter, said excess hydrofluoric acid giving said bath a pH of more than 1 and less than 6, the anions of said bath comprising essentially fluorides and borates, said bath producing said highly ductile nickel coating when operated at current densities of less than 250 amperes per square decimeter.

60 ETIENNE L. A. CAMIN.  
SVEN E. HYBINETTE.  
HERBERT B. TAYLOR.

#### REFERENCES CITED

65 The following references are of record in the file of this patent:

#### UNITED STATES PATENTS

Number Name Date  
2,313,756 Loose Mar. 16, 1943

#### OTHER REFERENCES

Transactions of the American Electrochemical Society, vol. 15 (1909), pages 464, 465; vol. 23 (1913), pages 145, 146, 147; vol. 39 (1921), pages 460-481; vol. 81 (1942), pages 213-229.